

June 11, 1968

V. F. ZACKAY ET AL

3,388,011

PROCESS FOR THE PRODUCTION OF HIGH STRENGTH STEELS

Filed Oct. 8, 1965



Fig. 2.



Fig. 1.

INVENTORS

VICTOR F. ZACKAY  
EARL R. PARKER

BY

*Robert G. Goodman*

ATTORNEY

1

3,388,011  
**PROCESS FOR THE PRODUCTION OF HIGH STRENGTH STEELS**

Victor F. Zackay, Berkeley, and Earl R. Parker, Orinda, Calif., assignors to the United States of America as represented by the United States Atomic Energy Commission

Filed Oct. 8, 1965, Ser. No. 494,284  
1 Claim. (Cl. 148—12.3)

**ABSTRACT OF THE DISCLOSURE**

To produce high strength alloy steel with high ductility, the steel is processed by a series of steps comprised of tempering, applying stress at an elevated temperature, cooling and post-tempering. The steel is strained at a temperature in the range from 150° F. to 900° F., cooled and then post-tempered. The elevated temperature strain aging results in a substantial increase in the yield strength, and a favorable shape of the stress-strain curve for good mechanical properties.

This invention relates to a method for increasing the yield strength of alloy steel while maintaining a relatively high degree of ductility. The invention described herein was made in the course of, or under, Contract W-7405-ENG-48 with the United States Atomic Energy Commission.

In the normal heat treating of steel, strength is sacrificed to retain high ductility. It has been generally considered that elevated temperature heat treating is incompatible with high strength due to heterogeneous nucleation. Such nucleation tends to occur most easily at lattice imperfections or discontinuities which produce precipitates at grain boundaries and forms sites at which cracks will propagate and spread, causing catastrophic failure of the steel. Therefore, a very fine uniform dispersion of precipitates is needed for very high strength and should come from a homogeneously nucleated precipitation reaction. Thus this invention is directed primarily to those alloy steels having a very fine microstructure. The precipitates in such steels act in several ways as barriers to dislocation movement, such as strong impenetrable non-coherent particles. The precipitates can also act as coherent or incoherent particles through which dislocations can pass, but only at stress levels beyond those required to move dislocations through the parent lattice.

Ductility and toughness in metals depend upon the behavior of dislocations. In a steel suitable for most usages, plastic flow must be able to redistribute a high local load around notches and other discontinuities before cracks can form. In conflict with this requirement of notch ductility is the fact that high strength can only be obtained in ductile materials if plastic flow is inhibited by barriers that restrict the movement of dislocations. Thus, high strength and good toughness are seemingly incompatible requirements and in general the strongest metals have tended to be brittle and ductile ones weak.

The present invention provides for the desirable combination of properties by a process which includes elevated temperature strain aging of high strength steels which have a high dislocation density and a fine martensitic microstructure. Such strain aging substantially increases

2

the yield strength, in some cases by a factor as high as 25%. This increase in strength is obtained without the concomitant decrease in ductility which is normal in some tempering operations. There is a slight decrease in ductility, as will be subsequently shown, but this decrease is of a relatively minor nature. In the case of the ausformed steel, ductility is still maintained above 10%. In general, those steels having over 200,000 p.s.i. tensile strength and 10% ductility are usually classified as high strength steels.

It is thought that the strain aging gives a high dislocation density and that the dislocations are pinned by the very fine dispersion. A large number of dislocations is necessary for high strength, and by close control of the temperature during the strain aging a very fine martensitic microstructure is maintained.

Therefore it is an object of this invention to provide steels having a highly desirable combination of properties.

A principal object of this invention is to provide a process for increasing the yield strength of an alloy steel while maintaining a substantial degree of ductility.

Another object of the invention is to provide a process whereby an alloy steel can be heat-treated to increase strength and toughness and still maintain ductility.

In general, the invention is applicable to quenched and tempered steels of the class having a fine grained martensitic microstructure. Stress is applied to the steel for a controlled time period, to effect a plastic strain in the range from about one-fourth percent to about five percent, while the steel is maintained at an elevated temperature but below that at which coalescing of precipitates would occur. The steel is then cooled and may subsequently be tempered if necessary.

In the practice of the invention the exact process conditions will differ for each alloy steel, but can readily be determined experimentally, examples being hereinafter described. Essentially, five parameters are varied in such a way to yield the optimum results. The five variables are:

- 40 (a) Pre-tempering temperature
- (b) Amount of strain
- (c) Strain rate
- (d) Temperature during strain
- (e) Post-tempering temperature

45 The pre-tempering and post-tempering are optional steps if the ductility and toughness of the steel is sufficient without tempering. The pre-tempering temperature is generally maintained at about 600° F., the temperature at about which iron carbides form, but in any case below the higher temperature, i.e. about 900° F. at which alloy carbides will form. Thus, the subsequent strain aging at an elevated temperature nucleates the alloy carbides that are still in solution. The amount of strain has an upper limit determined by the plastic limit of the steel and is about 5% for certain steels. The minimum strain which may be employed is the amount sufficient to form dislocations for nucleation sites to occur and is about  $\frac{1}{4}\%$  for certain other steels. Three differing strain rates  $1.35 \times 10^{-3}$  / sec.,  $1.35 \times 10^{-4}$  / sec. and  $1.35 \times 10^{-5}$  / sec. have been used

50 and the effect on product strength of the differing strain rates was found to be minimal. The temperature of the steel during the strain has a substantial effect on the final properties of the steel and may range from room temperature up to about 900° F. The straining temperature is

generally maintained below the post-tempering temperature. By an appropriate selection of the steps and process conditions within the foregoing general limits, the desired combination of strength and ductility is produced.

Two original steels which have been processed in ac-

5 differing strain rates. Comparison of Tables III and IV shows that the strain rate does not appreciably alter the results as compared to the effect of the strain temperature. However, in each case the yield stress and tensile stress is substantially increased.

TABLE III

[Conventional H-11 steel post-tempered at 900° F., strain rate=1.35×10<sup>-3</sup>/sec.]

|                                 |      |      |     |      |     |      |
|---------------------------------|------|------|-----|------|-----|------|
| Strain Temperature, ° F .....   | 70   | 300  | 450 | 600  | 750 | 900  |
| Yield Stress, K p.s.i. ....     | 330  | 299  | 312 | 323  | 321 | 296  |
| Tensile Stress, K p.s.i. ....   | 330  | 322  | 318 | 328  | 327 | 323  |
| Elongation, percent.....        | 1.78 | 4.9  | 4.4 | 4.8  | 5.5 | 7.6  |
| Reduction in Area, percent..... | 12.0 | 10.2 | 8.8 | 12.8 | 9.4 | 14.0 |

TABLE IV

[Conventional H-11 steel post-tempered at 900° F., strain rate=1.35×10<sup>-3</sup>/sec.]

|                                 |      |      |      |      |      |      |
|---------------------------------|------|------|------|------|------|------|
| Strain Temperature, ° F .....   | 70   | 300  | 450  | 600  | 750  | 900  |
| Yield Stress, K p.s.i. ....     | 332  | 308  | 326  | 323  | *319 | 289  |
| Tensile Stress, K p.s.i. ....   | 322  | 316  | 326  | 328  | *322 | 330  |
| Elongation, percent.....        | 1.9  | 8.3  | 3.6  | 2.7  | 6.1  | 5.8  |
| Reduction in Area, percent..... | 15.0 | 13.4 | 12.6 | 15.5 | 14.6 | 18.3 |

\*Plotted on Figure 1.

cordance with the invention had the following composition.

The superior properties of the H-11 steel processed by this invention relative to conventional H-11 steel are ap-

TABLE I

|                        | C   | Si   | Mn  | S    | P    | Cr   | V  | Mo   |
|------------------------|-----|------|-----|------|------|------|----|------|
| Conventional H-11..... | .40 | .85  | .33 | .015 | .011 | 5.06 | .5 | 1.28 |
| Ausformed H-11.....    | .40 | 1.60 | .25 | .008 | .011 | 5.00 | .5 | 1.40 |

The ausformed H-11 steel refers to conventional H-11 steel which has been processed in accordance with the teachings of U.S. Patent No. 2,934,463 to D. J. Schmatz et al., issued Apr. 26, 1960. The ausformed H-11 has a finer martensitic microstructure and a high dislocation density due to the severe deformation of the ausforming. The conventional H-11 was quenched and tempered.

The two steels had the following tensile properties prior to the elevated temperature strain aging step of the present invention.

TABLE II

|                        | Yield Stress, p.s.i. | Tensile Stress, p.s.i. | Elongation, percent |
|------------------------|----------------------|------------------------|---------------------|
| Conventional H-11..... | 230,000              | 303,000                | 8                   |
| Ausformed H-11.....    | 303,000              | 360,000                | 14                  |

The steel as processed was in the shape of ½" rolled rods, however, it is obvious that the process is applicable to a wide range of shapes including bar, sheet, rod, tube and the like.

Referring to Tables III, IV, V, VI and VII, representative results obtained by straining 2% at the specified elevated temperatures are shown. Table III and IV refer to conventional H-11 steel, post-tempered at 900° F. at two

30 parent from the stress-strain curves on the attached drawing, FIGURE 1. The lower curve is for H-11 steel quenched and tempered at 900° F. and tested at room temperature. The upper curve applies to H-11 steel, processed in accordance with this invention, which has been 35 quenched, tempered at 900° F., strained 2% at 750° F., post-tempered at 900° F., and subsequently tested at 70° F. As can be seen from the curves the yield stress (YS) increases from 230,000 p.s.i. to 319,000 p.s.i., and the tensile stress (TS) from 303,000 p.s.i. to 322,000 p.s.i. In 40 addition the shape of the curve for the strain aged steel is more desirable for engineering applications.

Referring to Tables III and IV it is seen that an upper limit to the temperature of strain aging conventional H-11 is indicated by the smaller increase in the yield stress obtained by strain aging at 900° F. When the steel 45 is strain aged at room temperature (70° F.) the yield stress increases, but the ductility is too low to be of structural use. Thus, it is indicated that the temperature of the steel during strain aging should be greater than room temperature.

50 Tables V, VI and VIII show representative results obtained by elevated temperature strain aging of ausformed H-11 steels, at three different strain rates and the various indicated tempering temperatures.

TABLE V  
[Ausformed H-11 steel post-tempered at 900° F., strain rate=1.35×10<sup>-3</sup>/sec.]

|                                 |      |      |      |      |      |      |
|---------------------------------|------|------|------|------|------|------|
| Strain Temperature, ° F .....   | 300  | 450  | 525  | 600  | 750  | 900  |
| Yield Stress, K p.s.i. ....     | 353  | 362  | 359  | 361  | 340  | 311  |
| Tensile Stress, K p.s.i. ....   | 381  | 375  | 379  | 377  | 386  | 393  |
| Elongation, percent.....        | 11.1 | 10.8 | 12.1 | 10.8 | 10.9 | 8.2  |
| Reduction in Area, percent..... | 20.2 | 23.2 | 18.5 | 19.0 | 19.0 | 32.0 |

TABLE VI  
[Ausformed H-11 steel, strain rate=1.35×10<sup>-4</sup>/sec.]

| Post-Tempering Temperature, ° F..... | 900  | 750  | 600  | 500  | 350  |
|--------------------------------------|------|------|------|------|------|
| Strain Temperature, ° F.....         | 300  | 450  | 525  | 600  | 750  |
| Yield Stress, K p.s.i. ....          | 350  | 362  | 351  | 399  | 410  |
| Tensile Stress, K p.s.i. ....        | 378  | 375  | 376  | 399  | 410  |
| Elongation, percent.....             | 10.0 | 9.5  | 11.1 | 5.35 | 2.6  |
| Reduction in Area, percent.....      | 19.5 | 13.5 | 26.0 | 33.0 | 25.0 |
|                                      |      |      |      | 19.0 | 21.0 |
|                                      |      |      |      | 30.0 | 30.0 |
|                                      |      |      |      | 28.0 |      |

TABLE VII  
[Ausformed H-11 steel post-tempered at 900° F., strain rate=1.35×10<sup>-3</sup>/sec.]

|                                 |      |      |      |      |      |      |
|---------------------------------|------|------|------|------|------|------|
| Strain Temperature, ° F.....    | 300  | 450  | 525  | 600  | 750  | 900  |
| Yield Stress, K p.s.i. ....     | 349  | 370  | 390  | 358  | 326  | 347  |
| Tensile Stress, K p.s.i. ....   | 381  | 374  | 390  | 375  | 386  | 380  |
| Elongation, percent.....        | 8.1  | 9.6  | 12.7 | 11.7 | 11.6 | 8.3  |
| Reduction in Area, percent..... | 12.4 | 18.7 | 27.0 | 27.8 | 37.0 | 40.0 |

As can be seen from Tables V, VI and VII the yield stress is substantially increased and approaches the values obtained for the tensile stress. The ductility in most cases remains above 10%, which as mentioned previously is considered essential for high strength applications. Although the initial ductility was 14%, the decrease in ductility to about 10% is not disadvantageous in view of the large increase in the yield stress.

In the stress-strain curves obtained from Ausformed H-11 steel, as shown in FIGURE 2, the lower curve shows a yield of 303,000 p.s.i. of Ausform steel tempered at 600° F. The upper curve, for Ausform steel processed in accordance with this invention, gives a curve with a better shape and a substantial increase in yield stress; from 303,000 p.s.i. to 402,000 p.s.i. The tensile stress also is increased from 360,000 p.s.i. to 400,000 p.s.i. The increased strength is obtained by strain aging the Ausform steel 2% at 300° F., with subsequent tempering at 600° F.

Considering now a typical example of the steps and process conditions with which the Ausform steel data of Table V to VII were obtained, the following procedures were utilized.

Ausform H-11 rods having the properties previously listed in Tables I and II were precision ground to

0.113±.001 inch in diameter and 1.125±.001 inches in length. The rods were then mounted in a hot testing jig with recording instruments to measure temperature and strain. As noted in Tables V to VII, three different strain rates were utilized;  $1.35 \times 10^{-3}$ /sec.,  $1.35 \times 10^{-4}$ /sec. and  $1.35 \times 10^{-5}$ /sec. The elongation of the specimen was sensed directly at the end of the specimen by a combination of a mechanical micrometer and a differential transformer. This eliminates possible errors due to thermal expansion of the extension rods.

10 After straining at the indicated elevated temperature, the specimens were air-cooled by a blower and then given the post-tempering treatment in a furnace controlled within  $\pm 5^\circ$  F.

15 After the post-tempering treatment, the bars were honed to a uniform diameter and finally pulled to destruction at room temperature on an Instron testing machine, and the tensile data in Tables V to VII obtained.

20 Three additional steels were tested. Their designation and compositions are shown in Table VIII. These steels were strain aged by packrolling at elevated temperatures. Both Ausform and quenched and tempered conditions of each steel were investigated. The changes in the yield and tensile strengths and the toughness are shown in Table IX.

TABLE VIII

|        | C    | Cr   | Mo   | V     | Ni   | Mn   | Si   |
|--------|------|------|------|-------|------|------|------|
| HY-TUF | 0.25 | 0.30 | 0.39 | ----- | 1.74 | 1.35 | 1.25 |
| D6AC   | 0.26 | 1.14 | 0.99 | 0.02  | 0.54 | 0.70 | 0.22 |
| 5M21   | 0.19 | 0.48 | 2.93 | ----- | 3.02 | 0.49 | 0.36 |

TABLE IX

|                  | Strain Temp., °F. | Tempering Temp., °F. | Yield Strength, K p.s.i. | Tensile Strength, K p.s.i. | Elongation, Percent in 1.4"' | Toughness, in.-lb./in. <sup>2</sup> |
|------------------|-------------------|----------------------|--------------------------|----------------------------|------------------------------|-------------------------------------|
| HY-TUF Ausformed | 302               | 302                  | 273                      | 277                        | 2.9                          | 928                                 |
|                  | 302               | 437                  | 273                      | 276                        | 2.9                          | 1,171                               |
|                  | 302               | 572                  | 272                      | 272                        | 2.8                          | 1,127                               |
|                  | 302               | 707                  | 254                      | 255                        | 3.7                          | 1,220                               |
|                  | 437               | 437                  | 244                      | 261                        | 4.3                          | 1,232                               |
|                  | 437               | 572                  | 257                      | 263                        | 4.3                          | 1,261                               |
|                  | 437               | 707                  | 233                      | 243                        | 3.6                          | 1,268                               |
|                  | 572               | 572                  | 265                      | 267                        | 4.3                          | 1,407                               |
|                  | 572               | 707                  | 246                      | 246                        | 3.6                          | 1,449                               |
|                  | 707               | 707                  | 242                      | 244                        | 3.6                          | 1,511                               |
| HY-TUF Quenched  | Unstrained        |                      | 221                      | 257                        | 5.0                          | 1,584                               |
|                  | 302               | 302                  | 197                      | 230                        | 6.4                          | 2,582                               |
|                  | 302               | 437                  | 198                      | 227                        | 5.7                          | 1,864                               |
|                  | 302               | 572                  | 214                      | 226                        | 5.7                          | 1,900                               |
|                  | 302               | 707                  | 210                      | 226                        | 5.7                          | 2,043                               |
|                  | 437               | 437                  | 219                      | 238                        | 5.7                          | 1,605                               |
|                  | 437               | 572                  | 232                      | 246                        | 6.4                          | 1,780                               |
|                  | 437               | 707                  | 221                      | 238                        | 5.0                          | 1,998                               |
|                  | 572               | 572                  | 224                      | 229                        | 4.3                          | 1,504                               |
|                  | 572               | 707                  | 219                      | 221                        | 5.0                          | 1,726                               |
| D6AC, Ausformed  | 707               | 707                  | 227                      | 231                        | 4.3                          | 1,066                               |
|                  | Unstrained        |                      | 186                      | 220                        | 7.1                          | 1,881                               |
|                  | 302               | 302                  | -----                    | 282                        | 2.9                          | 379                                 |
|                  | 302               | 437                  | -----                    | 276                        | 2.9                          | 432                                 |
|                  | 302               | 572                  | -----                    | 286                        | 2.9                          | 458                                 |
|                  | 302               | 707                  | 269                      | 270                        | 2.1                          | 504                                 |
|                  | 437               | 437                  | 266                      | 266                        | 2.9                          | 939                                 |
|                  | 437               | 572                  | 270                      | 270                        | 2.9                          | 881                                 |
|                  | 437               | 707                  | -----                    | 252                        | -----                        | 853                                 |
|                  | 572               | 572                  | 248                      | 260                        | 5.0                          | 1,104                               |
| D6AC, Quenched   | 572               | 707                  | 234                      | 243                        | 5.0                          | 1,190                               |
|                  | 572               | 707                  | 234                      | 241                        | 5.0                          | 1,047                               |
|                  | 707               | 707                  | 226                      | 265                        | 5.7                          | 1,467                               |
|                  | 302               | 302                  | 192                      | 221                        | 7.1                          | 1,978                               |
|                  | 302               | 437                  | 191                      | 217                        | 5.0                          | 1,756                               |
|                  | 302               | 572                  | 192                      | 210                        | 6.4                          | 1,738                               |
|                  | 302               | 707                  | 193                      | 215                        | 6.4                          | 1,835                               |
|                  | 437               | 437                  | 217                      | 229                        | 4.3                          | 1,741                               |
|                  | 437               | 572                  | 203                      | 222                        | 5.0                          | 1,407                               |
|                  | 437               | 707                  | 194                      | 212                        | 5.7                          | 1,450                               |
| 5M21, Ausformed  | 437               | 572                  | 216                      | 223                        | 3.6                          | 1,356                               |
|                  | 572               | 707                  | 205                      | 212                        | 4.3                          | 1,372                               |
|                  | 572               | 707                  | 207                      | 216                        | 5.0                          | 1,246                               |
|                  | 707               | 707                  | 190                      | 217                        | 5.0                          | 2,043                               |
|                  | 302               | 302                  | 267                      | 280                        | 5.0                          | 1,052                               |
|                  | 302               | 437                  | 267                      | 276                        | 3.6                          | 1,020                               |
|                  | 302               | 572                  | 257                      | 269                        | 5.0                          | 872                                 |
|                  | 302               | 707                  | 243                      | 252                        | 5.7                          | 904                                 |
|                  | 437               | 437                  | 235                      | 253                        | 5.0                          | 1,132                               |
|                  | 437               | 572                  | 220                      | 244                        | 5.0                          | 1,001                               |
| Unstrained       | 437               | 707                  | 221                      | 235                        | 6.4                          | 971                                 |
|                  | 572               | 572                  | 247                      | 263                        | 4.3                          | 916                                 |
|                  | 572               | 707                  | 232                      | 251                        | 5.0                          | 866                                 |
|                  | 707               | 707                  | 229                      | 245                        | 5.7                          | 847                                 |
|                  | Unstrained        |                      | 212                      | 256                        | 6.4                          | 1,121                               |

TABLE IX—Continued

|                     | Strain Temp., °F. | Tempering Temp., °F. | Yield Strength, K p.s.i. | Tensile Strength, K p.s.i. | Elongation, Percent in 1.4" | Toughness, in.-lb./in. <sup>2</sup> |
|---------------------|-------------------|----------------------|--------------------------|----------------------------|-----------------------------|-------------------------------------|
| 5M21, Quenched----- | 302               | 302                  | 176                      | 214                        | 7.1                         | 1,910                               |
|                     | 302               | 437                  | 185                      | 211                        | 7.1                         | 1,746                               |
|                     | 302               | 572                  | 181                      | 206                        | 7.1                         | 1,457                               |
|                     | 302               | 707                  | 186                      | 209                        | 6.4                         | 1,431                               |
|                     | 437               | 437                  | 200                      | 209                        | 5.7                         | 1,828                               |
|                     | 437               | 572                  | 193                      | 206                        | 6.4                         | 1,747                               |
|                     | 437               | 707                  | 190                      | 202                        | 6.4                         | 1,678                               |
|                     | 572               | 572                  | 209                      | 219                        | 4.3                         | 1,152                               |
|                     | 572               | 707                  | 196                      | 208                        | 5.0                         | 1,511                               |
|                     | 707               | 707                  | 171                      | 176                        | 7.1                         | 1,203                               |
|                     | Unstrained        |                      | 170                      | 212                        | 7.1                         | 2,236                               |
|                     | Unstrained        |                      | 172                      | 216                        | 7.1                         | 1,966                               |

Attention is particularly invited to the yield and tensile strength of the specimens strain aged at the various strain temperatures. Comparison with the unstrained steel shows a substantial increase in strength. Furthermore, the toughness tests indicate that the toughness or resistance to cracking of the strain aged steel is maintained at a high level.

While the invention has been described with respect to certain specific steels, it is apparent that it is applicable to a wide variety of steels and that many modifications are possible within the spirit and scope of the invention. For instance, it is possible to vary the steel composition to vary the properties obtained. Other methods of straining and differing strain rates at alternate rates may be utilized. Thus it is not intended to limit the invention except as defined by the appended claim.

What is claimed is:

1. A process for increasing the yield strength of a quenched and tempered high alloy steel mass having a martensitic grain size of about one half the size which would be obtained by the normal quenching of austenite to martensite, comprising:

- 15 (a) applying stress to said steel for a controlled length of time to effect a plastic strain of about  $\frac{1}{4}$  percent to about 5 percent, while maintaining said steel during said stress within a temperature range of 150 degrees Fahrenheit to about 900 degrees Fahrenheit,  
 20 (b) cooling said steel mass to room temperature, and  
 (c) post-tempering said steel by heating to a temperature within the range from 350 degrees Fahrenheit to 900 degrees Fahrenheit whereby the yield point is substantially increased.

#### References Cited

#### UNITED STATES PATENTS

- 3,230,118 1/1966 Tufts ----- 148—12  
 2,924,544 2/1960 Nachtman.

HYLAND BIZOT, Primary Examiner.

DAVID L. RECK, Examiner.

35 W. W. STALLARD, Assistant Examiner.